

# UNITED STATES PATENT OFFICE.

CLEMENS DÖRR, OF COLOGNE, GERMANY.

## PROCESS OF UTILIZING CARBONIFEROUS COLLIERY WASTE.

SPECIFICATION forming part of Letters Patent No. 703,696, dated July 1, 1902.

Application filed August 25, 1900. Serial No. 28,018. (No specimens.)

To all whom it may concern:

Be it known that I, CLEMENS DÖRR, a subject of the German Emperor, residing at Cologne, Empire of Germany, have invented certain new and useful Improvements in Processes of Utilizing Carboniferous Colliery Waste, of which the following is a specification.

The various branches of industry at the present time make increased requirements on the steam-producing capacity of coal. The quality of the latter should therefore be as pure—that is to say, as free from ash—as possible.

The object of the present invention is to obtain and utilize to a good purpose all the hitherto unused and in the original form unusable combustibles, so to say, hidden in the waste heaps and the like of collieries. To effect this, the waste is granulated as finely as possible, (this is the principal part of the process,) coarse sandstone being separated from it, if necessary, and is then thoroughly mixed up in some cases with an admixture of coal-slime, coal-dust, or the like or of sawdust, peat, brown coal, and such like combustible matter. In a loose condition or after having been formed into cakes or blocks by some suitable process the material can be used as fuel for any purpose.

A special advantage revealed by experiments is that the fuel burns with an intense continuous flame. Owing to its high specific weight the ash residue is of relatively small volume. Coal or fuel produced by this process does not cake or form slag.

The value and importance of the invention become most obvious when the following comparison is made between the combustible value of the materials used in their original form and of the combustible produced by the new process. It is assumed that the material taken from the waste and rubble heaps has in its original form no practically utilizable combustible value, while for the coal-slime a combustible value of ninety per cent. is fixed, although the latter also must be regarded as partly-valueless waste and partly waste of slight value.

| Combustible values—                           |                                            |                                                      |                                                                             |            | 50 |  |
|-----------------------------------------------|--------------------------------------------|------------------------------------------------------|-----------------------------------------------------------------------------|------------|----|--|
| of the materials used in their original form. |                                            | of the combustibles produced by the present process. |                                                                             |            |    |  |
| I.                                            |                                            |                                                      |                                                                             |            |    |  |
| 64.10 p.c.                                    | Coarse wash heap waste.                    | 0 p.c.                                               | Combustible value according to analysis by Mining Laboratory at Bochum.     | 63.20 p.c. | 55 |  |
| 32.05 p.c.                                    | Separated waste.                           | 0 p.c.                                               |                                                                             |            |    |  |
| 3.85 p.c.                                     | Resin, combustible value, max. 100 p.c.    | 3.85 p.c.                                            |                                                                             |            |    |  |
| 100.00 p.c.                                   | Combustible value.                         | 3.85 p.c.                                            |                                                                             |            | 60 |  |
|                                               |                                            |                                                      | Against this....                                                            | 3.85 p.c.  |    |  |
|                                               |                                            |                                                      | Combustible value gained.                                                   | 59.35 p.c. |    |  |
| II.                                           |                                            |                                                      |                                                                             |            |    |  |
| 80.40 p.c.                                    | Separated waste.                           | 0 p.c.                                               | Combustible value according to analysis by Mining Laboratory at Bochum.     | 83.60 p.c. | 65 |  |
| 11.76 p.c.                                    | Coal slime, comb. value, max. 90 p.c.      | 10.58 p.c.                                           |                                                                             |            |    |  |
| 3.92 p.c.                                     | Fine coal, combustible value, max. 95 p.c. | 3.72 p.c.                                            |                                                                             |            |    |  |
| 3.92 p.c.                                     | Hard pitch, comb. value, max. 100 p.c.     | 3.92 p.c.                                            |                                                                             |            | 70 |  |
| 100.00 p.c.                                   | Combustible value.                         | 18.22 p.c.                                           |                                                                             |            |    |  |
|                                               |                                            |                                                      | Against this....                                                            | 18.22 p.c. | 75 |  |
|                                               |                                            |                                                      | Combustible value gained.                                                   | 65.38 p.c. |    |  |
| III.                                          |                                            |                                                      |                                                                             |            |    |  |
| 61.00 p.c.                                    | Fine wash heap waste.                      | 0 p.c.                                               | Combustible value according to analysis by Dr. Karl Hohmann, of Düsseldorf. | 84.22 p.c. |    |  |
| 10.00 p.c.                                    | Coarse wash heap waste.                    | 0 p.c.                                               |                                                                             |            | 80 |  |
| 20.00 p.c.                                    | Coal slime, comb. value, max. 90 p.c.      | 18.00 p.c.                                           |                                                                             |            |    |  |
| 5.00 p.c.                                     | Pure coal, comb. value, max. 95 p.c.       | 4.75 p.c.                                            |                                                                             |            |    |  |
| 2.00 p.c.                                     | Dextrin, comb. value, max. 100 p.c.        | 2.00 p.c.                                            |                                                                             |            | 85 |  |
| 2.00 p.c.                                     | Colophony, comb. value, max. 100 p.c.      | 2.00 p.c.                                            |                                                                             |            |    |  |
| 100.00 p.c.                                   | Combustible value.                         | 26.75 p.c.                                           |                                                                             |            |    |  |
|                                               |                                            |                                                      | Against this....                                                            | 26.75 p.c. | 90 |  |
|                                               |                                            |                                                      | Combustible value gained.                                                   | 57.47 p.c. |    |  |

By the present process, therefore, highly valuable and rich supplies of combustible

matter which were hitherto regarded as los are opened up and utilized.

Having now particularly described and ascertained the nature of the said invention and 5 in what manner the same is to be performed, I declare that what I claim is—

The method of utilizing carboniferous colliery waste consisting in finely granulating such material, and adding thereto coal-slime,

coal-dust, small coke and the like, as herein 10 set forth.

In witness whereof I have hereunto set my hand in presence of two witnesses.

CLEMENS DÖRR.

Witnesses:

KARL SCHMITT,  
L. BARNES.